

## UNITED STATES PATENT OFFICE

THEODORE WILLIAMS DIKE, OF NEW WESTMINSTER, BRITISH COLUMBIA, CANADA,  
ASSIGNOR TO I. F. LAUCKS, INC., OF SEATTLE, WASHINGTON, A CORPORATION OF  
WASHINGTON

## PROCESS OF GLUING

No Drawing.

Application filed May 28, 1930. Serial No. 456,813.

In the usual methods of gluing, it is customary to employ a fluid or dispersed gluing material. This necessarily involves the introduction of a large amount of water for the conditioning of an adhesive of such type. All this water must then ultimately be eliminated. Aside from the disadvantages of thus having to introduce and eliminate a large volume of water, which is useless so far as adhesion proper is concerned, detrimental effects to the wood or the like also occur. Excessive swelling of the fiber, warpage and much checking are more or less inevitable concomitants. Objectionable staining of the wood is also common. On account of the limitations imposed by the liquid adhesive it has not been practical moreover to provide protective treatment other than by ultimate surface application to the finished product. A procedure making possible the avoidance of all of these drawbacks, and at the same time providing desired internal treatment of protective measures, irrespective of limitations of the gluing agent is of fundamental importance and highly desirable.

To the accomplishment of such objects and related ends, the invention, then, consists of the features hereinafter fully described and particularly pointed out in the claims, the following description setting forth certain illustrative embodiments of the invention, these being indicative of but a few of the various ways in which the principle of the invention may be employed.

In accordance with the invention, the materials to be glued, for instance elements for wood panels or ply-wood, are supplied with adhesive base, preferably in discrete particle form, and an addition agent for modifying the character of the product is included, with, or in any convenient order, as before or after the adhesive base, or both and the panel elements are assembled, and pressed.

As adhesive base material, I may employ the segregated proteins, such as casein, gluten, segregated or isolated protein from oil seed flours, such as soyabean, hempseed, castor, etc., or I may employ a vegetable proteinous material in the form of a ground seed flour, for instance the residue of oleaginous

seeds from which the oil has been removed being particularly advantageous. Examples of this are flour or meal made from cake or residue from soyabean, peanuts, cottonseed, flaxseed, perillased, hempseed, rapeseed, copra, tung nuts, castor beans, etc. In some instances I may employ a starch, also in un-dispersed condition. Readily dispersible proteins, such as blood albumen, animal glue, lactalbumin, etc. may be employed, also in discrete particle form, particularly where excessive penetration is suitably guarded against.

With the adhesive base in suitably divided or discrete particle form, as contrasted with dispersed or liquid glue, such material may be applied to the pieces to be glued conveniently by dusting or sprinkling. In the case of woods containing moisture, as green or wet material from a veneer cutter, it is merely necessary to apply the adhesive base in the dry powdered form. Where the moisture content of the wood is excessive it may be preliminarily reduced by suitable means. On the other hand, where the wood surfaces are dry, it is desirable to add a small amount of moisture. This may be done by brushing or spraying by an atomizer head or the like. The application of the moisture may precede or follow the application of the adhesive base. In some cases I may supply the moisture along with the adhesive, the adhesive then being in the form of a moistened or suspended mass, still, however, retaining its discrete particle form as distinguished from a dispersed or liquid condition. By "dispersion" of course is meant that colloidal condition in which the colloid is indefinitely disseminated homogeneously throughout the system.

With the adhesive base, or before its application or if preferred, after, or both, there is included also, as indicated, an addition agent. This may be an agent to supply water of crystallization, insolubilizing material, protective substances such as materials having a fireproofing action or biocidal action against fungi, bacteria, insects, etc.; for instance, barium hydroxide, a salt, such as sodium fluoride, a salt of a weak acid and

strong base such as a phosphate, sodium phosphate, sodium carbonate sodium metasilicate, ammonium phosphate, barium peroxide, bichromates, chrome alum, other alums, tannic acid, gallic acid, etc., sulphur compounds, as calcium thiocarbonate, or liquid and gaseous sulphur compounds, such as carbon disulphide, introduced in any suitable manner, for instance by adsorption in the adhesive 5 base or some convenient menstruum, copper salts, as copper chloride, copper sulphate, etc., phenol, creosote, cresylates, betanaphthol, alphanaphthol, camphor, oil of cedar, etc. As fireproofing agents, ammonium 10 phosphate as above noted, borax, etc. Soluble and hygroscopic compounds, such as caustic soda, may be dissolved in the moistening water and be thus applied.

Preferably, an agent to supply water or 20 crystallization, insolubilizing material, and fireproofing and biocidal ingredients are all employed together.

The minimum amount of moisture desirably present for the development of adhesion 25 where employing an adhesive base in discrete particle form as set forth, may range between about one-fourth to one and one-half times the amount of the dry adhesive base. Larger amounts up to the full moisture content of 30 green plies as coming from the veneer cutter are not detrimental to the formation of a satisfactory bond, but the presence of excess moisture increases the time required in the hot press proportionately to its presence. 35 When all the materials concerned are in a relatively dry state, satisfactory adhesion may be developed in some instances without the necessity of resort to heat, pressure alone being sufficient. The pressure employed may 40 vary depending upon the materials, soft materials, for instance a soft and open textured wood like cottonwood in the green undried state being satisfactorily handled with about forty pounds pressure per square inch, while 45 dense hard materials, for instance dry birch, may be treated at about 300 pounds pressure. The upper limit in any case would be determined by the possible crushing of the texture of the material. In the application 50 of heat where desired, temperatures of 160-375° F. may be had, the lower temperatures of around 160° being sufficient to set such an adhesive base as blood albumen, while the higher range of temperature is effective 55 in the insolubilizing of such adhesive bases as casein, oil seed flours, etc. Since the process avoids the large amount of water customarily handled in the wet gluing processes, it will be seen that it now becomes commercially 60 feasible to make up ply-wood in a single stage operation, bonding it together and drying it at the same time, thereby very greatly increasing plant capacity.

With dry wood the present process lends 65 itself particularly well to high speed gluing,

since there is no large excess of water to be eliminated, and very conveniently moisture requirements may be wholly or partly met by the incorporation of a compound having water of crystallization, such as the phosphates, 70 borax, barium hydroxide, etc. For example: 50 parts of casein are mixed with about 50 parts of trisodium phosphate. This is sprinkled upon a sheet of dry ply material, for instance as coming from the veneer drier, 75 another ply is superposed, the dry adhesive base is applied, and another ply is superposed. The assemblage is then subjected to pressure and heat in a press a temperature corresponding to a steam pressure of about sixty pounds 80 being adequate to set a  $\frac{1}{16}$  panel of gumwood in about one minute. This is an example illustrating gluing dry wood with a dry powdered adhesive base without applying any moisture as such to the assembly, the water 85 required for forming the bond being supplied by the water of crystallization contained in the addition agent.

Likewise with dry wood a strong and water resistant bond may be obtained with great 90 rapidity by applying to the ply about one part by weight of water by sprinkling, together with one part of the following adhesive base, combining a hydrolyzable sodium salt, a soluble barium compound, and 95 calcium hydroxide, said agents having a quick setting action upon proteinous materials and also an insolubilizing action, thus: 100 parts of soya bean flour, 20 parts of barium hydroxide, 10 parts of trisodium phosphate and 100  $1\frac{1}{2}$  parts of hydrated lime are mixed together. This is applied to the panel elements following the application of water, with superposition in succession, and the assembled panel is hot-pressed. With  $\frac{1}{16}$  face 105 plies a bond is formed in one minute with heat of the order of 60 lbs. steam pressure. By inclusion of beta-naphthol or oil of cedar with the oleaginous seed flour or other adhesive base in discrete particle form and ammonium 110 phosphate, a product may be had which is resistant against fungi and insects, as well as being fire resistant. In fact, in this manner combined ultimate structures may be had suitable for chest, closet and other construction 115 where it is desired to afford protective action against insects, etc., and such a product may be made much more effective than the usual cedar wood structures since the amount of protective agent incorporated in 120 the structure can assume such proportions as desired. The addition to the adhesive base of ammonium phosphate, beta-naphthol, oil of cedar, etc., may thus provide all-around 125 protection against hazards of fungi, insects, fire, etc., besides providing a wood product or the like in which the glue seams are characterized by a high strength and freedom from blistering and staining as well.

By supplying a biocide, fireproofing, or 130

other protective agent, for instance, sodium meta-silicate, ammonium phosphate, beta naphthol, alums, borax, para-formaldehyde, etc. in powdered form, these may be readily applied in admixture with the adhesive base and the procedure correspondingly simplified.

5 Wood and other materials capable of being bound together by an adhesive may thus be readily glued; with a corresponding absence of the obstacles characteristics of the old methods in which a large surplus of water had to be introduced and eliminated, nor is it necessary that the materials glued together be of definite geometrical shape.

10 This application is a continuation in part of my application Ser. No. 335,998, filed January 29, 1929.

15 The following applications are continuations in part of the present case: Serial No. 518,944, filed February 28, 1931; Serial No. 538,983, filed May 21, 1931; Serial No. 565,929, filed September 29, 1931; Serial No. 594,396, filed February 20, 1932; Serial No. 25 565,930, filed September 21, 1931, it being noted that claims specifying the use of a hydroxide of an alkali metal are included in the latter application.

20 Reference is also made to the following applications which are also continuations in part of said application Serial No. 335,998: Serial No. 454,832, filed May 22, 1930; Serial No. 455,977, filed May 26, 1930; Serial No. 455,978, filed May 26, 1930; Serial No. 35 456,814, filed May 28, 1930.

Reference is also made to the application of Theodore Williams Dike, Serial No. 596,070, filed March 1, 1932.

25 Other modes of applying the principle of my invention may be employed, change being made as regards the details described, provided the features stated in any of the following claims, or the equivalent of such, be employed.

30 I therefore particularly point out and distinctly claim as my invention:—

1. A process of gluing, which comprises applying to a surface to be incorporated an adhesive base in discrete particle form, supplying also an alkali metal compound, assembling, and pressing.

2. A process of gluing, which comprises applying to a surface to be incorporated an adhesive base in powdered form, supplying also in powdered form a material containing water of crystallization, assembling, and pressing.

3. A process of gluing, which comprises applying to a surface to be incorporated an adhesive base in discrete particle form, supplying also in powdered form an alkaline agent containing water of crystallization and assembling, and pressing.

4. A process of gluing, which comprises applying to a surface to be incorporated an ad-

hesive base in discrete particle form, supplying also barium hydroxide, assembling, and pressing.

5. A process of gluing, which comprises applying to a surface to be incorporated an adhesive base in discrete particle form, supplying also a protective agent in powdered form, assembling, and pressing. 70

6. A process of gluing, which comprises applying to a surface to be incorporated an adhesive base in discrete particle form and an insolubilizing agent containing combined water and in powdered form, assembling, and pressing. 75

7. A process of gluing, which comprises applying to a surface to be incorporated an adhesive base in discrete particle form, supplying also a biocidal agent in powdered form, assembling, and pressing. 80

8. A process of gluing, which comprises applying to a surface to be incorporated an adhesive base in discrete particle form, supplying also a fireproofing agent, assembling, and pressing. 85

9. A process of gluing, which comprises applying to a surface to be incorporated an adhesive base comprising soyabean flour and barium hydroxide, assembling, and pressing. 90

10. A process of gluing, which comprises applying to a surface to be incorporated an adhesive base in discrete particle form, supplying also a phosphate, and beta-naphthol. 95

11. A process of gluing, which comprises applying to a surface to be incorporated an adhesive base in discrete particle form, supplying also a phosphate, and oil of cedar. 100

12. A process of gluing, which comprises applying a proteinous material in discrete powdered form to a surface to be incorporated supplying also in powdered form an agent providing water of crystallization, assembling, and pressing. 105

13. A composite structure glued together by an adhesive base supplied in discrete particle form and identifiable as so supplied and including barium hydroxide. 110

14. A composite structure glued together by an adhesive comprising soya bean flour and barium hydroxide. 115

15. A composite structure glued together by a proteinous adhesive base supplied in discrete particle form and identifiable as so supplied and including a biocidal agent. 120

16. A composite structure glued together by a proteinous adhesive base supplied in discrete particle form and identifiable as so supplied and including a fire-proofing agent. 125

17. A process of gluing, which comprises applying a proteinous material in discrete particle form to a surface to be incorporated, supplying also a phosphate, assembling, and pressing. 130

18. A process of gluing, which comprises applying a proteinous material in discrete particle form to a surface to be incorporated, 135

- supplying also barium hydroxide assembling, and pressing.
19. A process of gluing, which comprises applying a proteinous material in discrete particle form to a surface to be incorporated, supplying also a biocide in powdered form, assembling, and pressing.
20. A process of gluing, which comprises applying a proteinous material in discrete particle form to a surface to be incorporated, supplying also a sodium compound, assembling, and pressing.
21. A process of gluing, which comprises applying a proteinous material in discrete particle form to a surface to be incorporated, supplying also oil of cedar, assembling, and pressing.
22. A process of gluing, which comprises applying to dry wood an adhesive base in powdered form and supplying also a material containing water of crystallization, assembling and subjecting to bonding conditions, without the addition of a liquid as such.
23. A process of gluing, which comprises applying to dry wood a mixture of an adhesive base in powdered form and a material containing water of crystallization, assembling and subjecting to bonding conditions, without the addition of a liquid as such.
24. A process of gluing, which comprises applying to dry wood a proteinous adhesive base in powdered form and a material containing water of crystallization, assembling and subjecting to bonding conditions; no liquid as such being supplied.
25. A process of gluing, which comprises applying to dry wood powdered casein and trisodium phosphate, assembling and subjecting to bonding conditions, no liquid as such being supplied.
26. A process of gluing, which comprises applying an adhesive base in discrete particle form to a surface to be incorporated, supplying also an insolubilizing agent and an independent protective agent, assembling and subjecting to bonding conditions.
27. A process of gluing, which comprises applying a powdered adhesive base to a surface to be incorporated, supplying also in powdered form an agent providing water of crystallization, an insolubilizing agent and a protective agent, assembling and subjecting to bonding conditions.
28. A process of gluing, which comprises applying a powdered adhesive base to a surface to be incorporated, supplying also in powdered form an agent providing water of crystallization, an insolubilizing agent and a biocide, assembling and subjecting to bonding conditions.
29. A process of gluing, which comprises applying to a surface to be incorporated an adhesive base and an alkali metal compound, both in powdered form, assembling and subjecting to bonding conditions.
30. A process of gluing, which comprises applying a mixture of an adhesive base and an alkali metal compound in powdered form, assembling and subjecting to bonding conditions.
31. A process of gluing, which comprises applying in powdered form a mixture of an adhesive base and an insolubilizing agent containing water of crystallization, assembling and subjecting to bonding conditions.
32. A process of gluing, which comprises applying a mixture of an adhesive base and a protective agent in powdered form, assembling and subjecting to bonding conditions.
33. A process of gluing, which comprises applying to a surface to be incorporated an adhesive base in discrete particle form and a phosphate of sodium and subjecting to bonding conditions.
34. A process of gluing, which comprises applying to a surface to be incorporated an adhesive base in discrete particle form and a phosphate of ammonium and subjecting to bonding conditions.
- Signed by me this 12th day of May, 1930. 90  
THEODORE WILLIAMS DIKE.
- 95
- 100
- 105
- 110
- 115
- 120
- 125
- 130